

## 1

3,717,455

STAINLESS FERRITE-AUSTENITIC STEEL  
Nils Erik Allan Hede, Lars Ivar Hellner, and Hans Elof Johansson, Karlskoga, Sweden, assignors to Aktiebolaget Bofors, Bofors, Sweden  
No Drawing, Filed Feb. 16, 1970, Ser. No. 11,777  
Claims priority, application Sweden, Feb. 18, 1969,  
2,228/69  
Int. Cl. C22c 39/20

U.S. CL. 75—128 N

1 Claim 10

### ABSTRACT OF THE DISCLOSURE

A process of producing a stainless ferritic-austenitic steel having high resistance to intercrystalline corrosion is disclosed. The process comprises adding to the steel titanium in such an amount that the quotient  $Ti_{rest}/C$  is at least 4.  $Ti_{rest}$  is the total titanium present minus the quantities consumed to form titanium nitride, titanium oxide or other titanium compounds. C is the total carbon content of the steel.

The present invention relates to a stainless ferritic-austenitic steel.

Applicant's U.S. patent application 823,744 describes the manufacture of a stainless ferritic-austenitic steel which is highly resistant to intercrystalline corrosion, the special characteristic features of the process being the addition of niobium (columbium) to a stainless ferritic austenitic steel in such quantities that the quotient  $Nb_{res}/C$  amounts to at least 8,  $Nb_{res}$  being the total niobium content minus the amount of niobium used to bind the nitrogen present in the steel to niobium nitride and C is the total carbon content of the steel.

The above patent application also discloses a number of stainless ferritic-austenitic steels of specific compositions which can be used to advantage when practicing said process to which the reader is referred for more detailed information on the methods used in testing the resistance of the steel to intercrystalline corrosion and the other factors regarding the steels known from the said patent,

## 2

A steel having the following composition has previously been disclosed:

|        | Percent |
|--------|---------|
| C max. | 0.05    |
| 5 Si   | 0.5     |
| Mn     | 0.5     |
| Cr     | 26      |
| Ni     | 6.5     |
| Mo     | —       |
| Ti     | 0.20    |

and the remainder iron.

With regard to the rule given in the following for the content of niobium and titanium, it should be noted that, when using conventional metallurgical processes, a steel of the type quoted will present a nitrogen content of about 0.04–0.06%. This means that the given percentage of nitrogen will be consumed to a very high degree in binding this nitrogen to titanium nitride, and that the amount of residual titanium present in the known steel will be insufficient to eliminate the intercrystalline corrosion in the following process.

The process of the present invention is mainly characterized in that the niobium addition taught by patent application Ser. No. 823,744 is replaced by a titanium addition, this change being effected in a manner whereby the quotient  $Ti_{rest}/C$  amounts to at least 4, wherewith  $Ti_{rest}$  is the total titanium content minus the amount of titanium consumed in binding the nitrogen found in the steel to titanium nitride.

It should be particularly noted that, since titanium has a much greater affinity to oxygen than has niobium, it cannot be ignored that a certain amount of titanium will be consumed in forming titanium dioxide. The aforementioned total quantity of titanium thus represents the titanium content after subtraction of the amount of titanium consumed in forming titanium dioxide.

Similarly to the manner described in patent application Ser. No. 823,744 a number of alloys have been tested, to show the conditions when niobium is replaced by titanium.

The compositions of the sample alloys are shown in Table 1.

TABLE 1.—CHEMICAL COMPOSITION OF TESTED STEELS

| Steel<br>number | Percentual content of— |      |      |      |     |      |      |      |       | $Ti_{tot}$<br>C | $Ti_{rest}$<br>C |
|-----------------|------------------------|------|------|------|-----|------|------|------|-------|-----------------|------------------|
|                 | C                      | Si   | Mn   | Cr   | Ni  | Mo   | Ti   | Nb   | N     |                 |                  |
| 1               | 0.058                  | 0.37 | 0.71 | 27.0 | 5.3 | 1.42 | —    | —    | 0.030 | 0               | 0                |
| 2               | 0.017                  | 0.57 | 0.84 | 25.8 | 8.0 | 1.57 | —    | —    | 0.047 | 0               | 0                |
| 3               | 0.085                  | 0.56 | 0.77 | 25.5 | 5.0 | 1.42 | 0.39 | —    | 0.018 | 4.6             | 3.9              |
| 4               | 0.059                  | 0.79 | 0.80 | 26.0 | 8.0 | 1.56 | 0.35 | —    | 0.048 | 5.9             | 3.2              |
| 5               | 0.018                  | 0.67 | 0.67 | 25.6 | 6.4 | 1.51 | 0.54 | —    | 0.052 | 30              | 20               |
| 6               | 0.025                  | 0.40 | 0.65 | 27.0 | 6.1 | 1.41 | —    | 0.90 | 0.030 | 136             | 27               |

<sup>1</sup>  $Nb_{tot}/C$ .

<sup>2</sup>  $Nb_{rest}/C$ .

NOTE.— $Ti_{rest}$  has in this instance been calculated as the total Ti content of the steel minus the amount of titanium needed to bind the nitrogen found in the steel to titanium nitride. The actual  $Ti_{rest}/C$  ratio is smaller, since  $TiO_2$  occurs in alloys 3, 4 and 5.

for instance the values of mechanical strength of the steels and the influence of other alloying substances included therein.

The present invention relates to the discovery that the niobium addition taught by U.S. patent application Ser. No. 823,744 can be replaced by an addition of titanium.

The alloys disclosed in Table 1 under 1, 2 and 6 have previously been tested and the result recounted in U.S. patent application Ser. No. 823,744.

The alloys listed in Table 1 were then tested for their ability to resist corrosion, by subjecting them to boiling 3% sodium chloride solution saturated with silver chlo-

ride for 24 hours, after first heat treating the steel samples in accordance with Table 2.

manner described for steel with additions of niobium. The results of these tests are shown in Table 3.

TABLE 3.—MECHANICAL PROPERTIES

| Steel number | Yield point,<br>kp./mm. <sup>2</sup> | Ultimate tensile strength,<br>kp./mm. <sup>2</sup> | Elongation ( $\delta_5$ ),<br>percent | Contraction,<br>percent | Impact toughness,<br>KCV, kp.m. | Austenitic content,<br>percent |
|--------------|--------------------------------------|----------------------------------------------------|---------------------------------------|-------------------------|---------------------------------|--------------------------------|
| 1-----       | 57                                   | 72                                                 | 27                                    | 63                      | 9                               | 25                             |
| 2-----       | 47                                   | 70                                                 | 34                                    | 71                      | 20                              | 45                             |
| 3-----       | 52                                   | 65                                                 | 27                                    | 60                      | 14                              | -----                          |
| 4-----       | 46                                   | 65                                                 | 31                                    | 70                      | 13                              | 40                             |
| 5-----       | 67                                   | 69                                                 | 26                                    | 67                      | 12                              | 17                             |
| 6-----       | 58                                   | 68                                                 | 23                                    | 59                      | 6                               | 24                             |

The results of the test are shown in Table 2.

TABLE 2.—CORROSION DATA FOR THE ALLOYS TESTED  
[The tests were conducted in boiling 3% NaCl solution saturated with AgCl for 24 hrs.]

| Heat treatment condition    |                       |                |                           |                |                       |                           |
|-----------------------------|-----------------------|----------------|---------------------------|----------------|-----------------------|---------------------------|
| 976 C., 1h.-600 C., 5 mins. |                       |                | 975 C., 1h.-600 C., 5 hr. |                |                       | 975 C., 1h.-800 C., 5 hr. |
| Steel No.                   | Weight loss (percent) | Type of attack | Weight loss (percent)     | Type of attack | Weight loss (percent) | Type of attack            |
| 1-----                      | 10                    | I              | 12                        | I              | 5.5                   | P+I                       |
| 2-----                      | -----                 | -----          | 13                        | I              | -----                 | -----                     |
| 3-----                      | -----                 | -----          | 12                        | I              | -----                 | -----                     |
| 4-----                      | -----                 | -----          | 14                        | I              | -----                 | -----                     |
| 5-----                      | 0.1                   | P              | 0.4                       | I              | 8.7                   | P                         |
| 6-----                      | 0.2                   | P              | 1.2                       | I              | 11                    | I                         |

NOTE.—P=spot attack; I=intercrystalline attack.

As can be seen from Table 1, steel 1, which corresponds to steel manufactured in accordance with SIS 2324 and to which no niobium or titanium was added, was the victim of strong intercrystalline corrosion after only five minutes, which resulted in a considerable loss in weight. Steels 2, 3 and 4, of which steels 3 and 4 have relatively low additions of titanium, show after a stay-time of five hours very high losses in weight caused by intercrystalline corrosion. The amount of titanium added to steel 5 was larger, which means that a quotient  $Ti_{rest}/C$  was obtained which was considerably higher than that of the steels 3 and 4 where the uncorrected quotient  $Ti_{rest}/C$  was 3.9 and 3.2 respectively. Steel 5 is given an uncorrected value of 20 for the  $Ti_{rest}/C$  quotient but it should be particularly noted that the values of  $Ti_{rest}/C$  given in Table 2 are uncorrected values and therefore much higher than the important actual values of  $Ti_{rest}/C$  for the individual steels 3, 4 and 5. Steel 5 with the higher content of titanium showed no intercrystalline corrosion and was only subject to spot corrosion. Special tests have shown that an actual quotient of  $Ti_{rest}/C=4$  or above when corrected for oxidation to titanium dioxide results in a steel which is not subject to intercrystalline corrosion after being disposed to the heat treatments disclosed in Table 2 and which is only liable to very moderate spot attack.

Tests have also been made to establish the strength properties of the steels, the tests being conducted in the

15 It is evident that steel 5, which is more favourable from the point of view of corrosion and which has a higher  $Ti_{rest}/C$  quotient, presents properties of strength which will correspond with corresponding values of the Nb-alloyed steel SIS 2324 designated 6, and with regard to impact toughness even higher values.

What is claimed is:

20 1. A stainless ferritic-austenitic steel having a high resistance to intercrystalline corrosion, consisting essentially of:

|                             | Percent   |
|-----------------------------|-----------|
| 25 Carbon -----             | 0.02-0.08 |
| Silicon, maximum of -----   | 0.5       |
| Manganese, maximum of ----- | 1.0       |
| Nitrogen -----              | 0.06      |
| 30 Chromium -----           | 24-27     |
| Nickel -----                | 5-7       |
| Molybdenum -----            | 1.3-1.8   |

35 titanium in such an amount that the fraction  $Ti_{rest}/C$  is at least 4 and not greater than 20,  $Ti_{rest}$  being defined as total titanium less the sum of the titanium required for the binding of the nitrogen present in the steel and the titanium used in forming any titanium oxide, and C referring to the total carbon content of the steel, with the balance iron.

40

## References Cited

## UNITED STATES PATENTS

|              |         |                |          |
|--------------|---------|----------------|----------|
| 2,693,414    | 11/1954 | Dunn -----     | 75-128 T |
| 2,758,025    | 8/1956  | Clarke -----   | 75-128 T |
| 45 3,337,331 | 8/1967  | Ljunberg ----- | 75-128 T |
| 2,083,524    | 6/1937  | Payson -----   | 75-128 T |
| 3,563,729    | 2/1971  | Kovach -----   | 75-128 W |
| 3,574,002    | 4/1971  | Haydean -----  | 75-128   |

50 HYLAND BIZOT, Primary Examiner

U.S. Cl. X.R.

75-128 T, 128 W

55